

March 14, 1972

S. M. KOVACH ET AL.

3,649,517

RESINS PREPARED FROM AROMATIC HYDROCARBONS

Original Filed Sept. 28, 1966



## INVENTORS

Stephen M. Kovach  
Ralph E. Patrick

BY Walter H. Schneider

**ATTORNEY**

1

3,649,517  
RESINS PREPARED FROM AROMATIC  
HYDROCARBONS

Stephen M. Kovach, Ashland, and Ralph E. Patrick, Flatwoods, Ky., assignors to Ashland Oil, Inc., Houston, Tex.

Continuation of application Ser. No. 582,754, Sept. 28, 1966. This application Dec. 29, 1969, Ser. No. 888,160  
Int. Cl. C08f 15/42

U.S. Cl. 208—22

8 Claims 10

## ABSTRACT OF THE DISCLOSURE

Polymer products are produced by distilling a full range dipolene to remove an overhead product boiling below about 140 to 160° F. and a bottoms product boiling above 245 to 250° F., and an intermediate product boiling between these two materials, the overhead and bottoms are combined, polymerized, and distilled to recover a resin boiling above 350° F., and the intermediate product is either hydrogenated or dehydrogenated and thereafter polymerized in at least one stage of polymerization and distilled to recover a resin product boiling above about 245° F.

The present invention relates to the production of resins from aromatic hydrocarbons and the products thereof. In a more specific aspect the present invention relates to the production of resins from normally liquid hydrocarbon mixtures containing aromatics, mono-olefins and diolefins and the novel products thereof. In a still more specific aspect the present invention relates to the production of resins from dipolene and the novel products thereof.

Normally liquid hydrocarbon mixtures containing aromatics, mono-olefins and diolefins are produced by a variety of well known processes. Such processes include the pyrolysis or cracking of crude petroleum or fractions thereof containing at least two carbon atoms such as ethane, propane, propylene, butane, natural gasoline, light straight run gasoline, straight run naphtha, kerosene, light cycle oils produced in the cracking of gas oils to produce gasoline, straight run gas oil, etc. These processes are carried out with or without the aid of catalysts and in the presence or absence of steam. Generally, the reaction temperature is in the neighborhood of about 1350 to 1550° F. and the pressure may be from 0 to 50 p.s.i.g. or higher. Such pyrolysis operations are generally carried out, primarily, for the production of ethylene. The pyrolysis of hydrocarbons to produce ethylene results in a normally gaseous product containing unsaturated hydrocarbons; including, ethylene, normally liquid hydrocarbons rich in unsaturated hydrocarbons including olefins and diolefins of varying boiling points and structures, and various aromatic hydrocarbons, as well as tar. The normally liquid hydrocarbons and tar obtained from this process are considered by-products. These by-products are removed by rapidly cooling the pyrolysis products, usually by quenching with water to a temperature of about 400° F. A viscous tarry material condenses out of the gas during the quenching operation. Gases from the quenching operation are then compressed and cooled and a liquid material boiling between about 100° and 360° F. condenses out of the gases during the compression-cooling operation. This last material is known as dipolene.

Dipolene fractions obtained in the manner set forth normally contain about two-thirds aromatics and one-third non-aromatics, the latter being mostly olefins and

2

diolefins. The aromatic portion consists mainly of benzene and toluene both of which are valuable in their own right and which are normally recovered. Such benzene-toluene concentration is usually accomplished by removal of the unsaturated compounds from the dipolene or by the removal of the aromatics selectively. Aromatic removal has heretofore been practiced by selective adsorption on materials, such as, silica gel, activated alumina, etc. However, such selective adsorption of aromatics is not effective since diolefins behave quite similarly to the aromatics. Generally, the removal of the unsaturated compounds is practiced commercially by hydrogenation or polymerization of the dipolene. Hydrogenation and polymerization to remove unsaturates from aromatics are also inefficient and produce little in the way of valuable products. Normally the hydrogenation of dipolene produces substantial amounts of mono-olefins which upon polymerization do not yield resins having any real value. Polymerization of dipolene is practiced commercially by either thermal or catalytic techniques. Thermal polymerization of the dipolene yields resin products which contain substantial amounts of cyclic diolefins and normally has no effect on the acyclic diolefins and tertiary mono-olefins present. On the other hand, catalytic polymerization of dipolene, under normal conditions of temperature, pressure and catalyst, yields resins containing substantial amounts of aromatics.

Another convenient source of aromatic hydrocarbons, particularly benzene and toluene is an aromatic light oil obtained by the high temperature carbonization of coal. The products of this carbonization are coke and the aromatic light oil. This light oil contains relatively high concentrations of unsaturates, sulfur and nitrogen compounds in addition to benzene, toluene and xylene. For example, a coal tar light oil boiling in the range of about 150–300° F. will contain, roughly, 85% benzene-toluene and about 15% unsaturates and impurities. Heretofore, the recovery of aromatics from coal tar light oils, particularly the recovery of benzene, has been effected by acid washing with sulfuric acid, benzene crystallization followed by acid washing, hydrotreating followed by solvent extraction with an aromatic-selective solvent or hydrotreating followed by high severity hydrocracking. Each of these treatments has been found to have its own peculiar drawbacks. For example, acid treating alone results in a benzene product of high purity with a high thiophene content. Benzene crystallization followed by acid washing will produce a product of high purity having a low thiophene content, but, by the same token, the recoveries of benzene are low. Hydrotreating followed by solvent extraction produces a high purity benzene product but is a costly process and coking problems in the preheater to the hydrotreater exist. The final technique of hydrotreating followed by high severity hydrocracking is a costly proposition because of the high pressures and high temperatures involved and at times such treatment does not produce specification grade benzene.

As previously indicated hydrogenation or polymerization of wide boiling range fractions of aromatic hydrocarbon mixtures, such as, dipolene and coal tar light oils, does not produce resins which are suitable for use as drying oils. There is either no drying oil production, as in the case of hydrogenation followed by conventional polymerization; or resins containing substantial amounts of aromatics are produced, as in the case of catalytic polymerization under conventional conditions; or, finally, resins containing cyclic diolefins result, as by thermal polymerization under conventional conditions.

The process of the present invention has been found to produce resins substantially free of aromatics or cyclic diolefins and which are, therefore, excellent drying oils.

The following specific examples will illustrate the present invention.

Referring to the drawings an aromatic feed mixture containing at least about 50% aromatics and less than about 50% non-aromatics, consisting essentially of olefins and diolefins is utilized. By way of specific example, dipolene obtained as a by-product in the thermal pyrolysis of gaseous hydrocarbons to produce ethylene will be referred to. This dipolene fraction comprises about 75% by volume of material boiling through the boiling range of toluene (about 230° F.) and about 25% by volume of material boiling above the boiling range of toluene. Of this material approximately 39.9% is benzene. This feed mixture is first fed through line 10 to a distillation column 12. In distillation column 12 the feed mixture is split into a heart cut having a boiling range of about 140 to 250° F. and preferably between about 160° and 245° F. Material boiling below about 160° F. is discharged from the column through line 14 while material boiling above about 245° F. is discharged through

10 line 14

20

toluene fraction may be fed to polymerization column 34. In polymerization reactor 34 the benzene-toluene fraction may be subjected to polymerization in the presence of an acidic, solid oxide catalyst, particularly boria-alumina and silica-alumina. Other such catalysts include silica-magnesia, fluoride promoted alumina, etc. The polymerization should be carried out at a temperature between about 0 and 300° F., and preferably 50° to 250° F. at a pressure between about 0 and 3000 p.s.i.g., preferably between about 0 and 1000 p.s.i.g., and at a liquid hourly space velocity (LHSV) between about 0.1 and 10, and preferably between about 0.5 and 5.

Table I below shows the results of a series of polymerizations of full range dipolene, containing 75% by volume of material boiling through the boiling range of toluene and 25% boiling above toluene, and the heart cut fraction of the present invention, containing 100% by volume of material boiling through the boiling range of toluene, respectively, utilizing both silica-alumina and boria-alumina catalysts.

TABLE I

| Run number          | 1                                                               | 2                                                | 3                                                | 4                                                               |
|---------------------|-----------------------------------------------------------------|--------------------------------------------------|--------------------------------------------------|-----------------------------------------------------------------|
| Feed                | Raw dipolene                                                    | Raw dipolene                                     | Heart-cut dipolene.                              | Heart-cut dipolene.                                             |
| Catalyst            | 10B <sub>2</sub> O <sub>3</sub> -Al <sub>2</sub> O <sub>3</sub> | SiO <sub>2</sub> -Al <sub>2</sub> O <sub>3</sub> | SiO <sub>2</sub> -Al <sub>2</sub> O <sub>3</sub> | 10B <sub>2</sub> O <sub>3</sub> -Al <sub>2</sub> O <sub>3</sub> |
| Temperature (° F.)  | 120                                                             | 120                                              | 160                                              | 160                                                             |
| Pressure (p.s.i.g.) | 0                                                               | 0                                                | 100                                              | 100                                                             |
| LHSV                | 2                                                               | 1                                                | 1                                                | 1                                                               |
| Product (percent):  |                                                                 |                                                  |                                                  |                                                                 |
| Benzene             | 39.0                                                            | 40.0                                             | 70.0                                             | 68.8                                                            |
| Toluene             | 28.0                                                            | 25.0                                             | 30.0                                             | 31.2                                                            |
| Resin               | 8.0                                                             | 10.0                                             | 10.5                                             | 10.5                                                            |
| >Toluene            | 25.0                                                            | 25.0                                             | 0.0                                              | 0.0                                                             |

line 16. The fraction boiling below benzene (about 160° F.) is combined with the fraction boiling above toluene (about 245° F.). These combined fractions are fed through line 18 to polymerization reactor 20. In polymerization reactor 20 the material is processed under select polymerization conditions to insure that no aromatics are incorporated into the resin product. These conditions, include, 0 to 3000 p.s.i.g. and preferably about 0 to 1000 p.s.i.g.; a temperature in the neighborhood of about 0 to 300° F. and preferably about 50 to 250° F.; and a liquid hourly space velocity of about 0.1 to 10 and preferably about 0.5 to 5.0. By way of specific example, a pressure of about 100 p.s.i.g., a temperature of about 200° F. and a LHSV of about 1.0 produce outstanding results. The catalyst is preferably 2 to 15% boria on alumina or silica-alumina. However, any acidic, solid oxide catalyst including silica-magnesia, fluoride promoted alumina, etc. can be used. The product of polymerization column 20 is discharged through line 22 and is in turn fed to distillation column 24. In distillation column 24 the material is processed to remove unconverted material and leave the desired resin as a distillation bottoms boiling below about 350° F. Accordingly, unconverted material is discharged through line 26 and the desired resin product through line 28. The resin yield obtained under the conditions set forth above was approximately 33% by volume of the total feed to distillation column 24 and is substantially free of aromatics. A single polymerization of this material is carried out since further processing leads to the production of olefin polymers and alkylated aromatics, apparently due to the absence of diolefins in the polymerization column. It appears that substantially complete removal of the diolefins occurs in column 20 during a single pass through the reactor.

The benzene-toluene cut boiling between about 160° and 245° F. is discharged from distillation column 12 through line 30. The benzene-toluene fraction can also be treated in several alternative fashions to produce additional amounts of aromatic-free resins.

One method of further treating the benzene-toluene fraction is by the selective polymerization of this fraction. Specifically, by opening valve 32 in line 30 the benzene-

35 It is clear from Table I that there is a net loss of aromatics when the full boiling range dipolene is treated and hence the resin product of this treatment will contain substantial amounts of aromatics. By way of contrast, aromatic recovery is essentially quantitative when the heart-cut of dipolene is polymerized, thus indicating that the resin product is substantially free of aromatics.

40 The polymerization product of column 34 is discharged to line 36 and is fed to distillation column 38 by opening valve 40. In distillation column 38 the product is separated into a fraction boiling below about 245° F. and a resin product boiling above about 245° F. The former product, which contains benzene and toluene, is fed to an appropriate benzene-toluene recovery operation through line 42 while the resin product boiling above about 245° F. is discharged through line 44. The resin product discharged through line 44 may be utilized as such, by withdrawing the same through line 46, or it may be combined with the resin product of polymerization column 29 by discharging the same through line 48. Where such blending is desired valve 50 would be closed and valve 52 would be open. The combined resin material would be fed to distillation column 24 where it would be further treated to recover a resin product boiling above about 350° F.

60 In another technique for recovering a valuable resin product from the benzene-toluene fraction being discharged through line 30, the heart cut mixture is first dehydrogenated in dehydrogenation reactor 54. For this purpose the benzene-toluene fraction is fed to column 54 through line 56 by closing valve 32 and opening valve 58. In dehydrogenation column 54 the heart cut fraction is dehydrogenated under conventional conditions to convert cyclohexadienes to aromatics. Suitable conditions for the operation of the dehydrogenator, include, the use of an active hydrogenation-dehydrogenation metal, including, those from Groups V-A, VI-A, VIII, I-B and II-B, on a neutral or basic support, such as alumina, silica, spinels, etc., for example, between about 0 and 500° F., and, preferably, 3 to 50% chromia on alumina, etc.; a temperature about 100-300° F.; a pressure of about 0 to 1000 p.s.i.g., and, preferably, about 0 to 100 p.s.i.g.; and

a liquid hourly space velocity of about 0.1 to 10, and, preferably, about 0.5 to 2. The product from dehydrogenation column 54 is discharged through line 60 and is passed to polymerization column 34, by opening valve 62 and feeding the material to line 64. In column 34 the dehydrogenated heart cut fraction is treated under essentially the same conditions previously set forth. After polymerization, the polymerizate passes to distillation column 38 where it is separated to recover the resin fraction boiling above about 245° F. Table II below shows the results of dehydrogenating a heart cut fraction. This heart cut fraction initially contained 10.5% <benzene, 76.0% benzene, 12.9% toluene and 2.7% >toluene. Of this feed about 2.7% were cyclohexadienes.

TABLE II

|                   |                                                                    |
|-------------------|--------------------------------------------------------------------|
| Feed              | Heart-cut dipolene.                                                |
| Catalyst          | 10Cr <sub>2</sub> O <sub>3</sub> -Al <sub>2</sub> O <sub>3</sub> . |
| Temperature, ° F. | 300.                                                               |
| Pressure p.s.i.g. | 0.                                                                 |
| LHSV              | 0.75.                                                              |
| Product:          |                                                                    |
| <Benzene          | 7.8                                                                |
| Benzene           | 78.5.                                                              |
| Toluene           | 13.3.                                                              |
| >Toluene          | 0.4.                                                               |
| Cyclohexadiene    | 0.1.                                                               |

Yet another method of recovering valuable resin products from the heart cut fractions passing through line 30 is by the hydrogenation of this material followed by polymerization. In this instance the heart cut fraction is charged to hydrogenation column 66 through line 68 which is controlled by valve 70. Hydrogen is supplied through line 72 and valve 74 from an external source not shown. Hydrogenation is, preferably, carried out in the presence of about 0.1 and 10% rhenium heptoxide on alumina as a catalyst. In the course of processing high sulfur feed materials the rhenium heptoxide will be converted to rhenium heptasulfide or its lower sulfides. The sulfide can also be produced prior to use of the catalyst by treating rhenium heptoxide with hydrogen sulfide. Other suitable catalyst, include, platinum or palladium on alumina, etc. The hydrogenation treatment is preferably carried out at a temperature of about 100 to 300° F. although temperatures from 75 to 400° F. can be used. A pressure in the range of zero to 3000 p.s.i.g. may be used, and preferably one between zero and 1000 p.s.i.g. The liquid hourly space velocity (LHSV) should be between 0.1 and 10, and preferably between 0.5 and 2, while a hydrogen rate between 100 and 1000 cubic feet per barrel of feed and preferably between 100 and 300 cubic feet is used. The hydrogenation product is discharged through line 76 by opening valve 78. From line 76 the hydrogenation product passes to line 64 and thence to polymerization column 34. From polymerization column 34 the polymerization product passes to distillation column 38 where it is treated in the same manner as previously described.

The following table illustrates the results of hydrogenating a heart cut dipolene, containing, 10.6% <benzene, 74.8% benzene, 14.1% toluene and 0.5% >toluene, and had a bromine # of 24.9.

TABLE III

|                                         |                                          |
|-----------------------------------------|------------------------------------------|
| Feed                                    | Heart cut dipolene.                      |
| Catalyst                                | 0.5% Re-Al <sub>2</sub> O <sub>3</sub> . |
| Temperature ° F.                        | 300.                                     |
| Pressure, p.s.i.g.                      | 0.                                       |
| LHSV                                    | 0.75.                                    |
| H <sub>2</sub> , ft. <sup>3</sup> /bbl. | 200.                                     |
| Product:                                |                                          |
| <Benzene, percent                       | 9.0.                                     |
| Benzene, percent                        | 75.0.                                    |
| Toluene, percent                        | 15.0.                                    |
| >Toluene, percent                       | 1.0.                                     |
| Bromine #                               | 11.1.                                    |

Yet another means of treating the heart-cut fraction passing through line 30 is by a combination of selective polymerization treatments. In this series of treatments the heart-cut fraction is treated in column 34 by the low severity polymerization treatment previously described. From column 34 the polymerization product is discharged through line 36 and thence to line 80. This material is fed to second polymerization column 82 by opening valve 84 in line 80. The small volumes of unsaturates remaining after polymerization in column 34 are primarily secondary olefins having normal or branch chains. Further polymerization of these olefins could be accomplished under severe conditions to effect complete olefin removal. However, such severe polymerization would normally lead to aromatic alkylation and a consequent loss of valuable benzene and toluene as well as contamination of the resin product. Accordingly, in column 82 the polymer product of column 34 is subjected to polymerization in the presence of an acidic solid oxide catalyst and a tertiary olefin. The tertiary olefin is introduced through line 85 and valve 86. When secondary olefins are treated with acidic catalysts they yield secondary carbonium ions which undergo aromatic alkylation as readily as polymerization. However, by introducing the tertiary olefin, tertiary carbonium ions are produced which drive the reaction toward polymerization rather than aromatic alkylation. In polymerization column 82 the catalyst may be any acidic solid oxide catalyst, silica-alumina, boria-alumina, silica-magnesia, fluoride promoted alumina, etc. and the tertiary olefin may be any olefin in the range of C<sub>4</sub> to C<sub>10</sub> and their dimers, especially isobutylene and isoamylene. Temperature conditions appropriate to this reaction are zero to 300° F. and preferably 50 to 200° F. The pressure should be maintained between 0 and 1000 p.s.i.g. and preferably between 50 and 200 p.s.i.g. The liquid hourly space velocity (LHSV) should be between 0.1 and 10 and preferably between 0.5 and 2. A tertiary olefin to feed ratio (volume/volume) of 1/1-1000 and preferably 1/10-100 should be utilized. A comparison of the polymerization of a fraction, boiling between 160 and 245° F., from a first polymerization treatment is shown in the following table, where the second polymerization was carried out with a silica-alumina catalyst, at 160° F., at 100 p.s.i.g. and at a LHSV of 1.0. This feed comprised; 12.6% <benzene, 73.2% benzene, 14.2% toluene and 0.0% >toluene.

The product of polymerization column 82 is discharged through line 88 and valve 90 and thence the distillation column 38 where it is further processed to separate the benzene-toluene fraction and the resin product boiling above about 245° F.

TABLE IV

| Run Number          | 1                                                | 2                                                |
|---------------------|--------------------------------------------------|--------------------------------------------------|
| Feed                | Heart cut from first polymerization.             | Heart cut from first polymerization.             |
| Catalyst            | SiO <sub>2</sub> -Al <sub>2</sub> O <sub>3</sub> | SiO <sub>2</sub> -Al <sub>2</sub> O <sub>3</sub> |
| Temperature (° F.)  | 200                                              | 200                                              |
| Pressure (p.s.i.g.) | 100                                              | 100                                              |
| LHSV                | 1                                                | 1                                                |
| Tertiary olefin     | None                                             | 1% isobutylene.                                  |
| Product (percent):  |                                                  |                                                  |
| <Benzene            | 8.6                                              | 5.6                                              |
| Benzene             | 77.0                                             | 79.6                                             |
| Toluene             | 15.0                                             | 15.0                                             |
| >Toluene            | 0.0                                              | 0.0                                              |

We claim:

1. A resin product obtained by distilling a hydrocarbon mixture selected from the group consisting of dipolene, having a boiling range of about 100-360° F., and coal tar light oil, having a boiling range between about 150 and 300° F., to remove a benzene-toluene concentrate, having a boiling range between about 160° F. and 245° F., recombining the fraction boiling below 160° F. and the fraction boiling above 245° F., subjecting said recombined fractions to polymerization in the presence of an acidic-solid oxide catalyst at a temperature of about 0° F. to 300° F. a pressure of about 0 to 3000 p.s.i.g., and a

liquid hourly space velocity between about 0.1 and 10, and distilling the polymerization product to recover a resin boiling above about 350° F.

2. A product in accordance with claim 1 wherein the hydrocarbon mixture is dipolene.

3. The product in accordance with claim 1 wherein the hydrocarbon mixture is coal tar light oil.

4. A resin product obtained by distilling a hydrocarbon mixture selected from the group consisting of dipolene having a boiling point between about 100° and 360° F., and coal tar light oil having a boiling point between about 150° and 300° F., to obtain a benzene-toluene concentrate, having a boiling range between about 160° and 245° F., subjecting said benzene-toluene concentrate to polymerization in the presence of an acidic, solid oxide catalyst at a temperature of about 0° to 300° F., a pressure of about 0 to 3000 p.s.i.g., and a liquid hourly space velocity of about 0.1 to 10; combining the fraction boiling below 160° F. and the fraction boiling above 245° F.; polymerizing said combined fractions in the presence of an acidic, solid oxide catalyst at a temperature of about 0 to 300° F., a pressure of about 0 to 3000 p.s.i.g., and a liquid hourly space velocity of about 0.1 to 10; combining the products of the first polymerization and the second polymerization steps; and distilling said combined products of said polymerization steps to recover a resin boiling above about 245° F.

5. A resin product obtained by distilling coal tar light oil having a boiling point between about 150° and 300° F., to obtain a benzene-toluene concentrate, having a boiling range between about 160° and 245° F., subjecting said benzene-toluene concentrate to polymerization in the presence of an acidic, solid oxide catalyst at a temperature of about 0° to 300° F., a pressure of about 0 to 3000 p.s.i.g., and a liquid hourly space velocity of about 0.1 to 10, and distilling the polymerization product to recover a resin boiling above about 245° F.

6. A resin product obtained by distilling a hydrocarbon mixture selected from the group consisting of dipolene having a boiling range of about 100 to 360° F., and coal tar light oil boiling between about 150° and 300° F., to obtain a benzene-toluene concentrate, having a boiling range of about 160° to 245° F., subjecting said benzene-toluene concentrate to dehydrogenation in the presence of an active hydrogenation-dehydrogenation metal deposited on a base selected from the group consisting of a neutral and a basic material at a temperature of about 0° to 500° F., a pressure of about 0 to 1000 p.s.i.g., and a liquid hourly space velocity of about 0.1 to 10, subjecting the dehydrogenation product to polymerization in the presence of an acidic, solid oxide catalyst at a temperature of about 0° to 300° F., a pressure of about 0 to 3000 p.s.i.g., and a liquid hourly space velocity of about 0.1 to 10; combining the fraction boiling below 160° F. and the fraction boiling above 245° F.; subjecting said combined fractions to a second polymerization in the presence of an acidic, solid oxide catalyst at a temperature of about 0° to 300° F., a pressure of about 0 to 3000 p.s.i.g., and a liquid hourly space velocity of about 0.1 to 10; combining the first and the second polymerization products; and distilling said combined products of said polymerization steps to recover a resin boiling above about 245° F.

7. A resin product obtained by distilling a hydrocarbon mixture selected from the group consisting of dipolene

having a boiling range of about 100° to 360° F., and coal tar light oil having a boiling range of about 150° to 300° F., to obtain a benzene-toluene concentrate boiling between about 160° and 245° F., subjecting said benzene-toluene concentrate to hydrogenation in the presence of hydrogen and a hydrogenation catalyst at a temperature of about 100° to 300° F., a pressure of about 0 to 3000 p.s.i.g., and a liquid hourly space velocity between about 0.1 and 10, subjecting the hydrogenation product to polymerization in the presence of an acidic, solid oxide catalyst at a temperature of about 0 to 300° F., a pressure of about 0 to 3000 p.s.i.g., and a liquid hourly space velocity of about 0.1 to 10; combining the fraction boiling below 160° F. and the fraction boiling above 245° F.; subjecting said combined fractions to a second polymerization in the presence of an acidic, solid oxide catalyst at a temperature of about 0 to 300° F., a pressure of about 0 to 3000 p.s.i.g., and a liquid hourly space velocity of about 0.1 to 10; combining the products of the first and the second polymerization steps; and distilling said combined products of said polymerization steps to recover a resin boiling above about 245° F.

8. A resin product obtained by distilling a hydrocarbon mixture selected from the group consisting of dipolene boiling between about 100° and 360° F., and coal tar light oil boiling between about 150° and 300° F., to obtain a benzene-toluene concentrate boiling between about 160° and 245° F., subjecting said benzene-toluene concentrate to polymerization in the presence of an acidic, solid oxide catalyst at a temperature of about 0° to 300° F., a pressure of about 0 to 3000 p.s.i.g., and a liquid hourly space velocity between about 0.1 and 10, subjecting the polymerization product to a second polymerization in the presence of a tertiary olefin from an external source, in a ratio of tertiary olefin to hydrocarbon mixture of about 1:1 to 1:1000, and in the presence of an acidic, solid oxide catalyst at a temperature of about 0° to 300° F., a pressure of about 0 to 3000 p.s.i.g., and a liquid hourly space velocity of about 0.1 to 10; combining the fraction boiling below 160° F. and the fraction boiling above 245° F.; subjecting said combined fractions to polymerization in the presence of an acidic, solid oxide catalyst at a temperature of about 0° to 300° F., a pressure of about 0 to 3000 p.s.i.g., and a liquid hourly space velocity of about 0.1 to 10; combining the polymerization products of the second and the third polymerization steps; and distilling said combined products of said polymerization steps to recover a resin boiling above about 245° F.

#### References Cited

##### UNITED STATES PATENTS

|           |        |                       |           |
|-----------|--------|-----------------------|-----------|
| 2,353,596 | 7/1944 | Shiffler et al. ----- | 260—683.4 |
| 2,733,284 | 1/1956 | Hamner -----          | 260—674   |
| 2,733,285 | 1/1956 | Hamner -----          | 260—674   |
| 2,798,866 | 7/1957 | Gordon et al. -----   | 260—82    |
| 2,894,937 | 7/1959 | Banes et al. -----    | 260—82    |

HERBERT LEVINE, Primary Examiner

U.S. Cl. X.R.

208—40; 260—82, 93.1